

March 27, 1951

W. GRACE

2,546,857

COVERING FABRIC FOR UMBRELLAS

Filed Dec. 17, 1949



INVENTOR

William Grace

BY

Benjamin Swedler  
ATTORNEY

## UNITED STATES PATENT OFFICE

2,546,857

## COVERING FABRIC FOR UMBRELLAS

William Grace, New York, N. Y.

Application December 17, 1949, Serial No. 133,649

3 Claims. (Cl. 139—383)

1

This invention relates to textile fabric coverings for umbrellas, which coverings have reinforced selvedge edges capable of withstanding the stresses exerted thereon by the stays of the umbrellas without weakening or fraying.

Umbrella fabric coverings having reinforced selvedge edges produced by folding over the longitudinal edges and adhesively securing the folded over edges by means of an adhesive tape, such as a rubberized tape, have been proposed. Such coverings have been found objectionable for a number of reasons, including among others, (1) the fabric must be made of a width to provide for the folded edge portions; this and the securing of the folded edges by means of a tape adds substantially to the expense of manufacturing the fabric, and (2) the folded edges add bulk to the edge portion of the umbrella covering resulting in some cases in an unattractive edge.

It is an object of this invention to provide an umbrella covering fabric having reinforced selvedge edges and this without entailing additional manufacturing steps, such as the folding of the edge portions or the securing of the folded edges by means of an adhesive tape.

It is a further object to provide an umbrella covering fabric of uniform thickness having reinforced selvedge edges which can readily and efficiently be loomed of single width, but preferably of a width equal to any desired multiple of the single width, and, when the multiple width web is cut into single widths, each single width strip is automatically formed with reinforced selvedge edges which have no tendency to ravel.

Other objects and advantages of this invention will be apparent from the following detailed description thereof.

In accordance with my invention the umbrella covering fabric is woven from cellulose acetate yarn and the warp threads of the selvedge edges are of nylon yarn. Thus, the fabric has nylon warp threads in the selvedge edge portions thereof which due to the great tensile strength of the nylon yarn impart strength to and reinforce the selvedge edges.

As the cellulose acetate yarn one may use any of the well known acetate rayon yarns, such, for example, as that sold under the trade-mark "Celanese" for use in making umbrella covering fabrics, which yarns are thermoplastic or fusible. The nylon yarn is a high tensile strength yarn made from artificial fiber forming linear condensation polyamides which may be derived from polymerizable monoaminocarboxylic acids and their amide forming derivatives, as well as from

2

the reaction of diamines with dicarboxylic acids or amide forming derivatives of dibasic dicarboxylic acids. The nylon yarn used as the warp threads of the selvedge edges is of the same or substantially the same gauge as the acetate threads forming the rest of the fabric.

In the accompanying drawing forming a part of this specification and showing for purposes of exemplification a preferred form of this invention without limiting the claimed invention to such illustrative instance,

Figure 1 is a plan view of a portion of a fabric web of double width which may be cut along the longitudinal median line to produce a single width umbrella fabric covering embodying my invention;

Figure 2 is a plan view of an umbrella fabric covering embodying my invention; and

Figure 3 is a vertical section on an enlarged scale as compared with the scale of Figures 1 and 2 taken in a plane passing through line 3—3 of Figure 2.

In Figure 2 of the drawing an acetate fabric 10 is shown having selvedge edges 11 and 12 in which 25 warp threads 13 of the selvedge edges 11 and 12 are of nylon. A body portion 14 of this fabric is composed of warp threads 15 and weft or filler threads 16 of cellulose acetate. The weft or filler threads 16 extend across the nylon warp threads 13 forming the selvedge edges 11 and 12.

In the illustrative but non-limiting example shown in Figure 2 each selvedge edge may be from  $\frac{1}{4}$ " to 1" wide, preferably from  $\frac{5}{8}$ " to  $\frac{3}{4}$ ", and the width of the fabric may be from 18" to 36". A width within this range is now commonly used in the umbrella industry to produce triangular shaped panels by cutting fabric along the dotted lines shown in Figure 2. Each selvedge portion 11 and 12 preferably contains about thirty nylon warp threads, although a larger or smaller number of such warp threads may be employed, if desired.

In the embodiment of the invention shown in Figure 1, the fabric is woven of double the desired width, i. e., as woven the fabric is from 36" to 52" wide with the selvedge edges 17 and 18 from  $\frac{1}{4}$ " to 1" wide and the centrally located intermediate longitudinally extending portion 19 from  $\frac{1}{2}$ " to 2" wide, preferably from  $1\frac{1}{4}$ " to  $1\frac{1}{2}$ " wide. The warp threads of the selvedge edges 17, 18 and of the intermediate longitudinally extending portion 19 are of nylon. The filler threads and the remaining warp threads of the fabric of Figure 1 are of cellulose acetate. The longitudinally extending portion 19 has its longi-

tudinal median line coincident with that of the fabric web and its width just double that of the selvedge edges 17, 18, so that, when the web is cut on the longitudinal median line, a single width web having selvedge edges of the same width as shown in Figure 2 results. While the web shown in Figure 1 is of double the desired width, it will be understood a fabric may be loomed in narrow looms of just the desired width or in looms forming any desired multiple of the desired width. In the latter case each interiorly disposed longitudinally extending portion corresponding to portion 19 of Figure 1 and along which the web is cut to form the selvedge edges of the single width strip is woven with nylon warp threads and is formed of a width double the width of the selvedge edges.

The cutting of the web is performed by a hot knife, such as a rotating knife maintained at a temperature of 650° to 750° F., usually about 700° F. The exact temperature of the knife depends on the speed of cutting. In the case of cutters operating at relatively high speeds the temperature thereof should be near the upper portion of the above noted range. For those operating at lower speeds the temperatures should be near the lower portion of this range. The cutting effects fusing of the ends of the cellulose acetate filler threads disposed across the nylon warp threads causing the cut edges of the filler threads to bond with the nylon threads, as indicated by the reference character 21, Figure 3. Ravelling of the cut edges is thus prevented.

Preferably, cutting of the fabric of the type shown in Figure 1 is effected before the fabric is shipped to the umbrella manufacturer; the product shipped to such manufacturer being that shown in Figure 2 in bolt or roll form. However, if desired, a web of double width, as shown in Figure 1, or even of a greater multiple width, may be shipped to the umbrella manufacturer, who in use would cut it longitudinally along the median line of the intermediate portion or portions having the nylon reinforcing threads either before or during the cutting into triangular shaped panels.

In the case of the production of a fabric embodying my invention in a single width loom, the edges of the filler threads are not fused to the nylon warp threads forming the selvedge edges, but are wound or woven thereabout so that they have no tendency to ravel.

It will be noted that this invention provides an umbrella fabric covering of uniform thickness having reinforced selvedge edges capable of withstanding the stresses to which the umbrella fabric is subjected in use by the umbrella stays due to raising and lowering of the umbrella, which fabric may be made in single or multiple width looms in any desired width, and which, when made on a multiple width loom with consequent economy in the manufacture of the fabric; and

thereafter cut into the desired width as hereinabove disclosed has no tendency to ravel or fray along the cut edges.

Since different embodiments of the invention could be made without departing from the scope of this invention, it is intended that all matter contained in the above description or shown in the accompanying drawing shall be interpreted as illustrative and not in a limiting sense.

What is claimed is:

1. An umbrella covering woven fabric of cellulose acetate warp and filler threads and having selvedge edge portions of equal width along the opposite edges thereof and at least one intermediate longitudinally extending portion of double the width of a selvedge edge portion, the warp threads in said selvedge edge and intermediate portions consisting of nylon.

2. A woven umbrella covering fabric from 36" to 52" wide of cellulose acetate warp and filler threads having selvedge edge portions of equal width along the opposite edges thereof, each approximately  $\frac{1}{4}$ " to 1" wide and having a centrally disposed longitudinally extending portion, the longitudinal median of which is coincident with the longitudinal median line of said fabric, said centrally disposed longitudinally extending portion being from  $\frac{1}{2}$ " to 2" wide, the warp threads in said selvedge edge portions and said centrally disposed longitudinally extending portion consisting of nylon.

3. A woven umbrella covering fabric from 18" to 26" wide comprising cellulose acetate filler threads, having a body portion in which the warp threads are composed of cellulose acetate and having edge portions of  $\frac{1}{4}$ " to 1" in width in which the warp threads are composed of nylon; one of said edge portions being a selvedge and the other of said edge portions having the ends of the filler threads fused to the nylon warp threads.

WILLIAM GRACE

#### REFERENCES CITED

The following references are of record in the file of this patent:

#### UNITED STATES PATENTS

| Number    | Name     | Date           |
|-----------|----------|----------------|
| 1,074,053 | Houser   | Sept. 23, 1913 |
| 1,089,857 | Muller   | Mar. 10, 1914  |
| 1,802,634 | Dreyfus  | Apr. 28, 1931  |
| 1,983,452 | Gwaltney | Dec. 4, 1934   |
| 2,035,138 | Maxfield | Mar. 24, 1936  |
| 2,145,715 | Dick     | Jan. 31, 1939  |
| 2,354,435 | Stedman  | July 25, 1944  |
| 2,400,327 | Womble   | May 14, 1946   |
| 2,501,213 | Cutler   | Mar. 21, 1950  |

#### FOREIGN PATENTS

| Country       | Date          |
|---------------|---------------|
| Great Britain | of 1891       |
| Great Britain | Jan. 21, 1926 |